

June 1, 1937.

H. VON FORSTER ET AL

2,082,557

INSULATING INSERT OF METAL

Filed Dec. 21, 1934



Inventors:  
Hermann Von Forster  
Rudolf Haefner  
By A. D. Weller  
Attorney

## UNITED STATES PATENT OFFICE

2,082,557

## INSULATING INSERT OF METAL

Hermann von Forster, Niederursel, near Frankfort-on-the-Main, and Rudolf Haefner, Frankfort-on-the-Main-Heddernheim, Germany, assignors to Vereinigte Deutsche Metallwerke Aktiengesellschaft, Frankfort - on - the - Main, Germany, a corporation of Germany

Application December 21, 1934, Serial No. 758,548  
In Germany December 23, 1933

6 Claims. (Cl. 72—127)

This invention relates to an insulating insert, specially intended for preventing the ascent of moisture, in building structures, such as foundation walls, pillars or the like, of masonry, concrete or the like. The present invention is an improvement over the internally insulated and water-proofed structure disclosed in U. S. Patent No. 2,030,417 granted to Hermann von Forster on February 11, 1936.

In contrast to the known insulating inserts of coatings of asphalt or tar, roofing felt or similar layers, the insert of the present invention consists of a comparatively thin band—for example 0.1—0.5 mm. thick—of ductile or forgeable corrosion-proof sheet metal, applied directly to the substratum that is to be protected (without any adhesive or other fixing layer), preferably by unrolling a continuous strip. The employment of such strips has the advantage that the number of joints, which are especially objectionable and detrimental to the insulation, is greatly reduced. Therefore, the walls or other structures to be protected can be covered with the insulating insert almost without leaving any interstices. It has been discovered that very thin sheeting, such as is 0.2 or 0.1 mm. in thickness, or even less, is sufficient for insulating purposes, provided that care be taken that the strip is quite compact in structure, that is to say impervious to moisture, on the one hand, and possesses mechanical strength on the other, so that the strip cannot suffer damage, either when being laid or when in position. This condition is fulfilled when the strip exhibits adequate properties in respect of strength and elongation. In this connection, special importance attaches to a sufficient capacity for deformation (drawing and forging) on the part of the metal employed, so that the thin strip of metal cannot be perforated by irregularities in the concrete or mortar substratum, projecting stones, particles of sand and the like, or by the pressure set up by the walls. Smooth and even metal strip that has been subjected for example, to an elongation or stretching treatment, and having straight longitudinal edges, has been found specially important for maintaining the impervious character of the insert.

The invention will be more fully understood by referring to the accompanying drawing which illustrates a vertical and fragmentary sectional view of a structure embodying the principles of the present invention.

Between a base A and a superstructure B both comprising brickwork C and layers of mortar D,

an insulating and water-proofing layer is provided constituted of thin metal sheet or strip E which is made of copper, copper alloys, nickel, nickel alloys, aluminum, aluminum alloys, or the like. As appears from the drawing, the insulating and waterproofing strip covers the full surface of the base and of the superstructure including the plaster F on the outer surface of the structure. The insulating metallic strip is in direct contact with the surface of both the base and the superstructure without the use of an adhesive. Due to its ductility, elasticity and strength, the metallic strip will exactly conform to the small depressions, elevations and other irregularities of the contacting structural surfaces without being perforated by the pressure of the superstructure and will provide a perfectly impermeable insulating and water-proofing layer.

Of course, the principles of the present invention may be embodied in structures of other types as, for example, of masonry, stonework, concrete, and the like, as those skilled in the art will readily understand.

In the case of insulation with layers of bitumen (such as asphalt board), the only method of attachment to pipes, gutters and other devices for carrying off water, is by cementing, which does not ensure perfect sealing. The conditions are difficult in the case of the insulating insert of the present invention, by means of which such connections can be effected without difficulty, in a permanently firm and durable manner, by lapping.

Since building materials such as cement, mortar, concrete and the like, contain substances—alkalis for example—which chemically attack metals, and may be leached out by ascending soil water or penetrative water that is under pressure, the metal strips employed must consist of metal that is as completely corrosion-proof as possible. Especially in the thin sheeting—which may be as little as 0.1 mm., or even less in thickness—that is used for the invention, the resistance of the insert to corrosion becomes of special importance. The insulating insert according to the present invention counteracts, in various ways, the difficulties arising in the employment of thin sheeting. Thus metals, such as nickel or nickel alloys, that resist the action of lyes, are preferably employed. It is true that metals of this kind are too expensive for general use, and are therefore applicable in special cases only, but when cheaper metals, such as copper, are employed for the strips, their resistance to

corrosion can be improved by alloying with other metals. Such alloying components comprise, for example, silicon, aluminium, nickel and tin. For example, copper-silicon alloys containing about 0.2-3% of silicon, copper-aluminium alloys containing about 0.5-10% of aluminium, and copper-nickel alloys containing about 0.5-30% of nickel have proved particularly suitable. The composition chosen for the alloy is preferably 5 such that protective layers retarding the progress of the attack are formed on the surface of the strip by the action of the substances excreted from the building structure. The employment of alloys certainly increases the cost of production of thin sheeting. The object of the present invention can, however, be more cheaply attained by providing metals of low resistance to corrosion with a coating of corrosion resistant metal, for example by electroplating copper strip 10 with nickel. In this case, chromium and other suitable metals can also be employed in place of nickel. The anti-corrosive layer can also be produced by spraying, plating or diffusion, instead of electrical deposition. A further possibility of protection also consists in providing the 15 said metal strips with protective coatings by oxidation or similar methods. Thus, a protective layer of oxide can be produced on copper strip by immersing same in molten saltpetre. Even a metal, such as aluminium, that offers but slight resistance to corrosion can be rendered suitable for the purposes of the invention by providing it with a coating of aluminium oxide, for example by oxidation. In place of a metallic 20 coating, non-metallic coatings also may be provided for protecting the metal strips. This method is generally the cheaper. Coatings of paint, lacquer and the like, protected by a covering layer, of paper, for example, are suitable for 25 this purpose. All these non-metallic coatings can be applied to one or both sides of the metal strip. In no case do they serve as an adhesive layer for attaching the metal strip to its sub- or super-stratum:

45 We claim:-

1. An insulated and water-proofed structure which comprises a base of brickwork, masonry, stonework, concrete and the like, an insulating and water-proofing layer constituted of a corrosion-resistant metal directly positioned on said base, and a superstructure above and in direct contact with said insulating layer, said metal strips being from about 0.1 mm. to about 0.5 mm. in thickness and having sufficient ductility 50 and strength to conform to irregularities of the surface of said base and said superstructure without being perforated.

2. An insulated and water-proofed structure which comprises a base of brickwork, masonry, stonework, concrete, and the like; an insulating and waterproofing layer constituted of long, foldable and corrosion-resistant metallic sheets of foil thickness directly positioned on said base; said sheets being thin enough to be ductile and 55 to conform to elevations and depressions of the

surrounding structural members and having sufficient mechanical strength to resist penetration of said structure; and a superstructure positioned on and in direct contact with said insulating layer.

3. An insulated and water-proofed structure which comprises a base of brickwork, masonry, stonework, concrete and the like; an insulating and water-proofing layer constituted of long, foldable metallic sheets of foil thickness directly positioned on said base; a corrosion-resistant protective coating on said metallic sheets; said sheets being thin enough to be ductile and to conform to elevations and depressions of the surrounding structural members and having sufficient mechanical strength to resist penetration of said structure; and a superstructure positioned on and in direct contact with said insulating layer.

4. An insulated and water-proofed structure which comprises a plurality of members of the structure made of brickwork, masonry, stonework, concrete, and the like, having a small space therebetween; and an insulating and water-proofing layer provided in said space consisting of long, rollable metallic sheets of foil thickness constituted at least partly of nickel and in direct contact with said structural members; said sheets being thin enough to be ductile and to conform to elevations and depressions of the surrounding structural members and having sufficient mechanical strength to resist penetration of said structure.

5. An insulated and water-proofed structure which comprises a plurality of members of the structure made of brickwork, masonry, stonework, concrete, and the like, having a small space therebetween; and an insulating and water-proofing layer provided in said space consisting of long, rollable metallic sheets of foil thickness constituted at least partly of copper and in direct contact with said structural members; said sheets being thin enough to be ductile and to conform to elevations and depressions of the surrounding structural members and having sufficient mechanical strength to resist penetration of said structure.

6. An insulated and water-proofed structure which comprises a plurality of members of the structure made of brickwork, masonry, stonework, concrete, and the like, having a small space therebetween; an insulating and water-proofing layer provided in said space consisting of long, rollable metallic sheets of foil thickness constituted at least partly of aluminum and in direct contact with said structural members; and a corrosion-resistant layer of aluminum oxide on at least one side of said sheets; said sheets being thin enough to be ductile and to conform to elevations and depressions of the surrounding structural members and having sufficient mechanical strength to resist penetration of said structure.

HERMANN VON FORSTER.  
RUDOLF HAEFNER.